

## UNITED STATES PATENT OFFICE

2,377,106

LUBRICANT AND PROCESS FOR PREPARING  
AND USING SAMEMaurice Reswick, Wilkinsburg, Pa., assignor to  
Standard Oil Development Company, a cor-  
poration of DelawareNo Drawing. Application October 29, 1942,  
Serial No. 463,780

8 Claims. (Cl. 252—56)

This invention relates to a novel lubricant and to methods of preparing and using same. More particularly, it relates to a metal fabricating lubricant and especially to one which is adapted for lubrication of sheet steel, etc., as it is being processed in high speed cold rolling mills. The product of this invention is intended to be used also as a replacement for palm oil which has largely been used heretofore by the steel mills for such purposes.

In the cold rolling of steel sheets and strip on the modern 4-Hi mills, it is necessary to use a lubricant to reduce the friction between the work rolls and the metal. The pressures and temperatures are high and experience has shown that palm oil is the best lubricant when heavy reductions in gauge are made. The usual procedure is to heat the palm oil in a tank, pump it to the rolling mill stands and apply it to the top and bottom rolls by means of a spray. A characteristic of palm oil is that it is a solid or a semi-solid at room temperatures but when heated to over 120° F. it becomes a fluid. When sprayed on the water-cooled rolls the palm oil congeals and is not washed off. During the rolling operation it spreads evenly over the surface of rolls, thus providing lubrication over the entire width of the sheet rolled.

The primary object of the present invention is to provide a metal fabricating lubricant which so nearly resembles palm oil in physical and chemical properties that in actual commercial operations in the steel mills where it is vitally important to have a high speed sheet steel lubricant having exactly the right combination of viscosity, lubricity, adhesiveness, and melting point or fluidity that it will be a completely satisfactory replacement for palm oil in commercial steel rolling practice.

Another object of this invention is to provide a lubricant which can also be used satisfactorily for other metal-fabricating processes such as cold drawing of metal, stamping and forming required when dies and presses are used.

Broadly, the invention comprises compounding or blending a foots oil, a petrolatum having a melting point of 90 to 130° F., a heavy mineral oil having a viscosity of 100—350 seconds Saybolt at 210° F., a fat such as hydrogenated fish oil, tallow, etc., and a fatty acid such as hydrogenated fish

oil acids and/or higher fatty acids such as stearic acid and oleic acid.

It is preferred that the foots oil be obtained from a paraffinic crude petroleum although other crudes such as naphthenic or mixed base crudes may be used if necessary. The heavy mineral oil may be derived from any available crude. Foots oil, which usually contains about 45%—50% of wax having a melting point of from 100 to 120, usually has a pour point of about 90° F.

The preferred fat to be used is a hydrogenated fish oil such as that marketed under the trade name of "Hydrofol Tinfat 50." Other fats or fatty materials which may be used are: degras, animal tallow, hydrogenated vegetable fats, such as of cottonseed oil, etc.

The preferred fatty acid for the purposes of this invention is a hydrogenated fish oil acid such as marketed under the trade name of "Hydrofol Acid 51," although other high molecular weight organic acids, in addition to those mentioned above, may be used such as cottonseed oil acids, stearic acid, palmitic acid.

In compounding these various ingredients, it is 25 of course understood that some variations may be made in the proportions of materials but generally the compositions selected should be within the following range of proportions:

30 Foots oil 40 to 60% preferably 45 to 55%  
Petrolatum 5 to 30% preferably 15 to 25%  
Heavy mineral oil 5 to 25% preferably 10 to 15%  
Fat 5 to 20% preferably 10 to 15%  
Fatty acid 2 to 20% preferably 5 to 15%

For the sake of illustration but without intending to limit the invention specifically to the precise materials and proportions used, the following examples are given:

| Material           | Examples |    |    |    |    |    |    |
|--------------------|----------|----|----|----|----|----|----|
|                    | 1        | 2  | 3  | 4  | 5  | 6  | 7  |
| Foot oil           | 50       | 50 | 55 | 50 | 40 | 40 | 50 |
| "Hydrofol Tinfat"  | 10       | 10 | 5  | 10 | 15 | 10 | 20 |
| "Hydrofol Acid 51" | 10       | 10 | 10 | 5  | 15 | 20 | 10 |
| Crude petrolatum   | 15       | 20 | 10 | 25 | 5  | 10 | 15 |
| Cylinder oil       | 15       | 10 | 20 | 10 | 25 | 20 | 5  |

In the above Examples 1 and 2, the materials

used had the following identifying characteristics:

Foots oil—

|                                        |          |    |
|----------------------------------------|----------|----|
| Pour point                             | ° F.     | 70 |
| Wax content (110 M. Pt.)               | per cent | 48 |
| Oil content (80 secs. vis. at 100° F.) | per cent | 52 |

Hydrofol Tinfat—

|                      |      |     |
|----------------------|------|-----|
| Melting point        | ° F. | 130 |
| Saponification value |      | 190 |
| Iodine value         |      | 10  |

Hydrofol Acid 51—

|                   |      |     |
|-------------------|------|-----|
| Saponification No |      | 194 |
| Acid No.          |      | 194 |
| Iodine No.        |      | 6   |
| Titre             | ° C. | 52  |

Crude petrolatum, melting point ° F. 130

Cylinder oil—

|                       |         |      |
|-----------------------|---------|------|
| Vis., Saybolt 100° F. | seconds | 3200 |
| Vis., Saybolt 210° F. | do      | 155  |

The finished compounded product identified above as Example 1 had the following characteristics:

|                                         |          |      |
|-----------------------------------------|----------|------|
| Melting point, A. S. T. M.              | ° F.     | 102  |
| Solidification point (A. S. T. M. pour) | ° F.     | 95   |
| Flash point                             | ° F.     | 370  |
| Fire point                              | ° F.     | 395  |
| Saybolt viscosity at 130° F.            | seconds  | 93   |
| Saybolt viscosity at 210° F.            | do       | 47   |
| Unworked penetration at 77° F.          |          | 182  |
| Worked penetration at 77° F.            |          | 284  |
| Saponification No                       |          | 40.9 |
| Free fatty acid (as oleic acid)         | per cent | 10.4 |
| Iodine value                            |          | 15   |

Both Examples 1 and 2 were used in large scale tests on a 54" cold roll tandem mill where normally steel sheets are reduced from 0.070" to 0.010" in commercial high speed rolling of sheet steel using rolling speeds such as 1500 to 3000 ft. per minute, and both of these products gave satisfactory results, although the product of Example 2 containing a slightly higher percentage of petrolatum and slightly less cylinder oil was slightly superior to Example 1.

The product of Example 2 was also used successfully on a 5 stand tandem mill, in rolling an extremely tough high-phosphor steel from an initial gauge of .072" to sheets having a finished gauge of .010", 32" wide, and rolled at a speed of 1700 ft. per min.

Undoubtedly the extremely satisfactory results obtained with the metal-fabricating lubricants of this invention are due to the cooperation of the various ingredients with one another to produce precisely the desired balance of physical and chemical properties which is so important and in fact actually critical for rolling sheet steel at such high speeds as those of 1500 ft. per minute and higher. Therefore it is probably impossible to ascribe any one particular characteristic of the finished product to one particular ingredient and say that that ingredient is solely responsible for such characteristic. However, in a general way, to assist those skilled in the art in making slight adjustments in the proportions of materials within the general range as indicated above as permissible, the following tentative explanation of the properties and functions of the individual constituents will be given.

The function of the foots oil as one of the principal components is to act as a vehicle for the other ingredients. Foots oil is a by-product in the manufacture of petroleum waxes and consists

of a mixture of a low viscosity oil and a low melting point wax. The desirable feature of foots oil is that the low viscosity oil is ideal for high speed rolling operations, which now go up as high as 3000 ft. per minute. The wax content of foots oil imparts to the compound a high cold test so that it acts in this respect in the same manner as palm oil.

Hydrofol Tinfat is a hydrogenated fish oil containing less than 20% of acids of C<sub>20</sub> to C<sub>22</sub>, the balance being mostly C<sub>18</sub> to C<sub>16</sub>, and it is suitable for lubrication at high temperatures. It has a low iodine number and in this respect it is superior to common tallow.

Hydrofol Acid 51 is also a hydrogenated fish oil similar to the Hydrofol Tinfat with the glycerides removed. The purpose of this fatty acid is to lower the surface tension of the compound and improve its wetting ability, causing it to spread quickly over the metal surfaces.

The crude petrolatum helps to make the product more adhesive to metal surfaces and both the petrolatum and the cylinder oil, such as that marketed under the name Cylesso 155, is used to impart to the compound a homogeneous structure, especially to break up the crystalline or granular structure due to the wax content in the foots oil.

The product of this invention is characterized by being a normally solid metal-fabricating lubricant which has a relatively low melting point since it becomes liquid at a temperature of about 90° F.-140° F., preferably about 95-110° F. and it reverts to a solid when the temperature is lowered about 5 to 10° F. below the melting point. It usually should have a viscosity of about 40-60 seconds, preferably 45-55 seconds Saybolt at 210° F. It also has good adhesion to the steel rolls and to the sheet metal being rolled. It may be applied to the rolls of a sheet metal rolling mill either by spraying or dripping from one or more suitably spaced tubes so as to provide even distribution of the lubricant throughout the entire length of the rolls. If desired, it may also be sprayed or run on to the sheet metal itself prior to, during or after rolling. Ordinarily this lubricant is heated to a temperature of about 150° to 175° F. in a suitable supply tank from which it is pumped to the various mill stands, where it may be applied, for instance, to the top and bottom back-up rolls. As the warm liquid lubricant impinges on the relatively cool roll surface, the liquid lubricant loses its fluidity, becoming more viscous and the copious flow of cold water, also usually applied to the rolls, assists in cooling the lubricant without washing it off, so long as the pressure of the water stream is not high enough to actually shear it off. When the sheet metal such as thin sheet steel actually goes through the work rolls, it becomes coated with the lubricant, but at the same time it is subjected to mechanical working during the reduction in thickness and at the contact area of the work rolls with the sheet strip, the temperature of the strip becomes sufficiently high to change the water into a cloud of steam and to liquefy the lubricant in a thin film, which assists in carrying the lubricant over to the next pass as a thin film on the rolled sheet metal.

If desired, this lubricant may be used in admixture with palm oil, such as in blends containing 50%, 25%, 10%, etc. of palm oil, especially until the workmen in the mills become accustomed to using it in place of the palm oil used heretofore.

It may also be emulsified with water before use, if desired.

The quantity of this roll lubricant to be used will, of course, vary according to various factors such as the mill design, the number of roll stands, the thickness gauge at the start and finish of the rolling and how much reduction is made in each individual pass, the surface finish desired, the method of application to the rolls and sheet metal, etc. Generally, however, the amount of oil used will be about 5 to 10 lbs. per ton of steel strip, generally a relatively small amount being required on the first stand and the largest amount being required on the next to the last stand or the one immediately preceding it. This same lubricant is well adapted for use as a rust inhibitor after the roller sheet steel has gone through the pickling bath to remove oxide scale. It may also be used to cover the molten metal bath during the manufacture of tin plate and terne plate.

In order to avoid waste this metal-fabricating lubricant may be recovered for re-use by a relatively simple system of salvaging and reconditioning. This involves merely collecting the oil, which is generally mixed with water and perhaps dust and fine iron scale particles, in a trench or sump under the cold roll mills, pumping the mixture from there, preferably through a  $\frac{1}{2}$ -inch mesh screen, into a settling tank, heating it under slight superatmospheric pressure, if desired to a temperature at least as high as  $150^{\circ}$  F. and preferably somewhat higher such as  $200^{\circ}$  and  $250^{\circ}$  F. in order to settle out the water and coarse foreign particles, and then drawing off the clarified oil. If desired, this clarified oil may be further refined by centrifuging.

I claim:

1. A normally solid lubricant having a melting point between about  $90^{\circ}$  F. and  $140^{\circ}$  F., a viscosity of about 40 to 60 seconds Saybolt at  $210^{\circ}$  F., comprising at least 60% by weight of foots oil and petrolatum, said lubricant also comprising about 5-40% of fatty material selected from the group consisting of fats and higher fatty acids.

2. A normally solid metal-fabricating lubricant having a melting point between about  $90^{\circ}$  F. and  $140^{\circ}$  F., a viscosity of about 40 to 60 seconds Saybolt at  $210^{\circ}$  F., comprising about 40-60% by weight of foots oil, said lubricant also containing about 10-30% of petrolatum, about 5-25% of heavy mineral oil having a viscosity of about 100 to 350 seconds Saybolt at  $210^{\circ}$  F., about 5-20% of a fat and about 2-20% of a higher fatty acid.

3. A normally solid metal-fabricating lubricant

having a melting point between about  $95^{\circ}$  F. and about  $110^{\circ}$  F., a viscosity of about 45 to 55 seconds Saybolt at  $210^{\circ}$  F. comprising about 40-60% by weight of foots oil, about 15-25% of petrolatum, about 5-25% of heavy mineral oil having a viscosity of 100 to 300 seconds Saybolt at  $210^{\circ}$  F., about 5-20% of a fat and about 2-20% of a higher fatty acid.

4. A normally solid metal-fabricating lubricant having a melting point between about  $95^{\circ}$  F. and about  $110^{\circ}$  F., a viscosity of about 45 to 55 seconds Saybolt at  $210^{\circ}$  F., comprising about 45-55% by weight of foots oil, about 15-25% of petrolatum, about 10-15% of heavy mineral oil having a viscosity of about 100 to 350 seconds Saybolt at  $210^{\circ}$  F., about 10-15% of a fat and about 5-15% of a higher fatty acid.

5. A normally solid metal-fabricating lubricant having a melting point between about  $95^{\circ}$  F. and about  $110^{\circ}$  F., adapted for cold rolling of sheet steel at a speed of at least 1500 feet per minute, comprising about 45-55% by weight of foots oil having a pour point of about  $70^{\circ}$  F. to about  $90^{\circ}$  F. and containing about 45-50% of wax having a melting point of from  $100^{\circ}$  F. to  $120^{\circ}$  F., said lubricant also containing about 15-25% of petrolatum having a melting point of about  $90^{\circ}$  F. to  $130^{\circ}$  F., about 10-15% of heavy mineral oil having a viscosity of about 100 to 350 seconds Saybolt at  $210^{\circ}$  F., about 10-15% of hydrogenated fish oil and about 5-15% of hydrogenated fish oil acids.

6. A normally solid metal-fabricating lubricant having a melting point between about  $95^{\circ}$  F. and about  $110^{\circ}$  F., adapted for cold rolling of sheet steel at a speed of at least 1500 feet per minute, comprising about 50% by weight of foots oil having a pour point of about  $70^{\circ}$  F. to about  $90^{\circ}$  F. and containing about 48% of wax having a melting point of from  $100^{\circ}$  F. to  $120^{\circ}$  F., in 52% of an oil having a viscosity of about 80 seconds Saybolt at  $100^{\circ}$  F., said lubricant also containing about 20% of petrolatum having a melting point of about  $90^{\circ}$  F. to  $130^{\circ}$  F., about 10% of a cylinder oil having a viscosity of about 3200 seconds Saybolt at  $100^{\circ}$  F. and about 155 seconds Saybolt at  $210^{\circ}$  F., about 10% of a hydrogenated fish oil acid.

7. Lubricant according to claim 6 in which the hydrogenated fish oil is "Hydrofol Tinfat."

8. Lubricant according to claim 6 in which the hydrogenated fish oil acid is "Hydrofol Acid 51."

MAURICE RESWICK.